

1

3,492,707

**METHOD OF PRODUCING ELASTIC FABRICS**  
Hiroyuki Segawa, Kurashiki, Japan, assignor to  
Kurashiki Rayon Co., Ltd., Kurashiki, Japan, a  
Corporation of JapanNo Drawing. Filed Feb. 12, 1968, Ser. No. 704,550  
Claims priority, application Japan, Feb. 16, 1967,  
42/10,003

Int. Cl. D01d 11/06; D02g 3/32

U.S. Cl. 28—75

7 Claims

**ABSTRACT OF THE DISCLOSURE**

A method of producing elastic products having beautiful appearance, which comprises applying an aqueous solution of polyvinyl alcohol to the surface of polyurethane elastic filaments, subjecting the filaments to drying under the stretched state to obtain easily controllable polyurethane elastic filaments having low elongation and high Young's modulus, making a woven or knitted product from said filaments together with ordinary hard fiber yarns, and treating the resulting product with hot water of 60–100° C.

This invention relates to a method of producing elastic woven fabrics and knitted goods in which are used the polyurethane continuous elastic filaments.

In general, the polyurethane continuous elastic fiber has a high elongation of as much as several hundred percent and an extremely low Young's modulus (as expressed in terms of its tenacity at 50% elongation) on the order of 0.01–0.2 gram per denier. As a consequence, in the various after treatments such as in twisting it with the other hard fiber yarns, its tension control is difficult. Hence, there tends to occur irregularities in the end product due to the fluctuation in tension such that at times it becomes practically impossible to produce the intended product.

As a result of having researched into the possibility of a method of temporarily setting the elongation of the polyurethane elastic filaments, we found according to this invention that the polyvinyl alcohol aqueous solution was most suitable as a treatment medium of the polyurethane elastic filaments and that by using this aqueous solution a pasting set effect of the elastic filaments in their stretched state could be obtained, with the consequence that a temporarily low elongation and a temporarily high Young's modulus for the elastic filaments could be obtained. Further, it was found that when the so treated polyurethane continuous elastic filaments and hard fiber yarns (e.g., nylon, polyester, etc.) are used and woven fabrics or knitted goods are made and thereafter the so obtained woven or knitted products whose elasticity is under restraint are relaxed using hot water, the polyvinyl alcohol which had been used for paste setting of the filaments is removed and at the same time the elastic filaments themselves whose elongation had been in a temporarily set state up to this time become relaxed and shrink, whereby elasticity develops in the woven or knitted products.

An object of this invention is to temporarily effect the lowering of the elongation of a polyurethane elastic filaments while, on the other hand, raising their Young's modulus to thereby provide a polyurethane continuous elastic filaments the management of which is simplified during their after-treatments. Another object is to provide a new method of producing high quality, fine looking woven or knitted products composed of the polyurethane continuous elastic yarns and hard fiber yarns.

Accordingly, this invention is directed to a method of producing elastic woven and knitted products which comprises applying to the surface of polyurethane continuous

2

elastic filaments an aqueous solution of polyvinyl alcohol having a degree of saponification of 50–100% followed by subjecting the filaments at least to drying under a stretched state ranging from at least 150% of their original length to below their breaking elongation to thereby obtain polyvinyl alcohol-coat low elongation polyurethane continuous elastic filaments having a elongation of not greater than 100% and a Young's modulus [expressed in terms of tenacity (g./d.) at 50% elongation] of at least 0.4 gram per denier, and thereafter making a woven or knitted product using the so obtained yarns and hard fiber yarns followed by treating said woven or knitted product with hot water of 60–100° C.

As the method of applying the aqueous solution of polyvinyl alcohol of a degree of saponification of 50–100% to the surface of the polyurethane continuous elastic filaments, any of the customarily practiced procedures may be employed in the invention method, such as the method of dipping the elastic filaments in the polyvinyl alcohol aqueous solution, the method of spraying the filaments with the polyvinyl alcohol aqueous solution, or the method of passing the filaments between rollers whereby the polyvinyl alcohol solution is imparted to the filaments when the latter passes between the rollers. Of these, the most convenient and desirable is however the dipping method.

According to the invention, it is an indispensable condition that the polyurethane continuous elastic filaments which have been applied the polyvinyl alcohol aqueous solution, as hereinabove indicated, are dried under a stretched state ranging from at least 150% of their original length to below their breaking elongation. A coating of polyvinyl alcohol is formed on the surface of the polyurethane continuous elastic filaments by this drying in the stretched state, and this demonstrates the effect of paste setting the filaments in their stretched state. Thus, the polyurethane continuous elastic filaments of high elongation and extremely low Young's modulus are converted into polyvinyl alcohol-coated low elongation polyurethane continuous elastic filaments having an elongation of not greater than 100% and a Young's modulus [expressed in terms of tenacity (g./d.) at 50% elongation] of at least 0.4 gram per denier. These filaments have the advantage that they are very easily managed in the subsequent after treatment steps. Further, as hereinafter described, in the various modes of practicing the invention, it is possible to add the stretching and heat treatment steps modified in various ways as well as to make various modifications in the temperature conditions during the polyvinyl alcohol application and drying operations.

In carrying out the stretching of the polyurethane continuous elastic filaments in the range from at least 150% of their original length to below their breaking elongation, the spun filaments immediately after their spinning may be drawn prior to the application of the polyvinyl alcohol aqueous solution, or the stretching of the filaments may be performed after having applied the polyvinyl alcohol aqueous solution to the spun filaments or, alternatively, the application of the polyvinyl alcohol aqueous solution and the stretching may be carried out simultaneously. While the stretching can be carried out at any temperature from room temperature to a temperature just below the decomposition point of the polyurethane continuous elastic filaments, usually a range between room temperature and 100° C. is to be preferred. The temperature of the polyvinyl alcohol aqueous solution is conveniently 0–60° C. from the operations standpoint, but after the application the dry heat treatment is preferably carried out at 60–100° C. By means of this dry heat treatment, not only the removal of the water on the surface of the polyurethane continuous elastic filaments is carried out but also their heat treatment is concurrently accomplished.

On the other hand, when a temperature of 60-100° C. is used for the polyvinyl alcohol aqueous solution, the drying may be carried out at from room temperature to 100° C. for removing the water on the surface of filaments. This drying step or the drying and heat treatment should be carried out in all cases under tension. In practicing the invention method, it is preferred that the polyurethane continuous elastic filaments are provided a thermal history ranging from 60° C. to a temperature just below the decomposition point of the filaments, and preferably from 60-100° C., during at least a certain period before the completion of the step of drying in a stretched state the polyvinyl alcohol applied to said polyurethane filaments, since such a thermal history has desirable heat treatment effects on the elastic filaments.

Further, after the drying of the polyurethane continuous elastic filaments, it is preferred that their cooling be carried out by holding the filaments at a temperature, e.g. room temperature, under free tension. By operating in this manner, the distortion of the residual elongation decreases and thus a shrinkage on the order of several percent to 10% occurs in the filaments.

In applying the polyvinyl alcohol aqueous solution to the polyurethane continuous elastic filaments, the first step of the invention, the amount of the polyvinyl alcohol to be adhered to the filaments, on a dried basis, is 5-200% by weight, and preferably 10-100% by weight, based on the filaments.

When the amount adhered of the polyvinyl alcohol is less than 5% by weight, the paste setting effect, one of the objectives of the invention, is not demonstrated fully, whereas when the amount adhered exceeds 200% by weight, the treated filaments become too thick, and difficulties are experienced in carrying out after treatment operations such as spinning. Hence, the amount adhered of the polyvinyl alcohol should preferably be held within the foregoing range.

The polyvinyl alcohol to be used in the invention is one whose degree of polymerization is 300-4000, and preferably 1000-3000, while its degree of saponification is 50-100%, and preferably 80-100%. The degree of saponification, as here used, denotes the saponification degree of polyvinyl acetate in the production of polyvinyl alcohol therefrom. Accordingly, the above-mentioned degree of saponification of 50% indicates that 50% of the acetyl groups in polyvinyl acetate have been converted to the hydroxyl groups by hydrolysis. The concentration of the aqueous solution of polyvinyl alcohol should be 1-30% by weight, and preferably 5-20% by weight.

The polyurethane continuous elastic filaments of the invention are obtained by spinning in customary manner the polyurethane polymer obtained by the reaction of a polymer glycol having a melting point of not more than 80° C., with an organic diisocyanate and the various chain extenders. While as the spinning method the various methods of such as the dry-spinning, melt-spinning and wet-spinning methods can be employed, in the herein-after given examples the polyurethane continuous elastic filaments obtained by the dry and wet-spinning methods will be described.

As the polymer glycols, useable are the polyether glycols, polyester glycols and polyetherester glycols.

Suitable polyether glycols include such as polyethylene glycol, polypropylene glycol, polytetramethylene glycol, polyhexamethylene glycol and the copolymers of these.

As the polyester glycols, suitable are the polycondensation products of the dicarboxylic acids such as succinic, adipic and sebacic acids with the low molecular weight glycols such as ethylene glycol, propylene glycol and butylene glycol.

The polyetherester glycols include the polycondensation products of the dicarboxylic acids, such as previously described, with such as diethylene glycol, triethylene glycol and tetraethylene glycol.

As the organic diisocyanates, useable are the polymethylene diisocyanates such as ethylene diisocyanate and hexamethylene diisocyanate, cycloalkylene diisocyanates such as cyclohexane 1,4-diisocyanate, and the diisocyanates containing an aromatic nucleus, such as tolylene diisocyanate, biphenylene 4,4'-diisocyanate, diphenylmethane 4,4'-diisocyanate and 1,5-naphthylene diisocyanate.

On the other hand, the chain extenders to be used in the diamine compounds such as hydrazine, ethylene diamine, tetramethylene diamine, hexamethylene diamine, 1,5-naphthylene diamine and p-phenylene diamine, amino alcohols such as ethanolamine and aminoethylmethanolamine, glycols such as ethylene glycol, propylene glycol, 1,4-butanediol and 1,5-pentanediol, and water.

According to the invention, the so obtained polyurethane continuous elastic filaments of low elongation and high Young's modulus are made into woven or knitted products by their conjoint use with the other hard fiber yarns. The hard fiber yarns, as here used, include all the usual filament yarns or spun yarns composed of natural or synthetic high molecular weight substances, as contrasted with the elastomers, and they are exemplified by such as polyester filaments, polyamide filaments, polyacrylonitrile yarns, polyethylene filaments, viscose rayon and cotton fiber yarns. Further, these hard fiber yarns may be also those which have been imparted the bulky treatment.

In the process of making the woven or knitted products using the polyurethane continuous elastic filaments of low elongation treated according to the invention and the other hard fiber yarns, a blended yarn, core yarn, twisting yarn, etc., of the aforesaid two fibers can be first made and then the woven or knitted products be made therefrom; or the end product can be obtained by using the polyurethane continuous elastic filaments of low elongation in their as-obtained form and directly weaving or knitting these filaments with the hard fiber yarns. Again, in making the woven or knitted products, it is also possible to use for either the warp or weft the polyurethane continuous elastic filaments, while using for the other the hard fiber yarns. These woven or knitted products, as used in the invention, may be any of those forms which are conventional. In this process of making the woven or knitted products, the various apparatuses, which are usually used in the processing of the hard fibers, can be used without modification, because the polyurethane continuous elastic filament treated according to the invention have a low elongation and a high Young's modulus. Thus there is the advantage that there is no need for any special tension controlling apparatus. Further, since the treated polyurethane continuous elastic filament excel in their form stability, there is no need to stretch the elastic filaments to an excessive degree in the yarn doubling step and the process of making the woven or knitted products. Hence, there is no possibility of the unevenness of tension. Consequently, the surface condition of the resulting woven or knitted products is uniform and they are in possession of a fine appearance.

According to the invention method, the woven or knitted products of various forms, obtained as hereinbefore described, must be treated with hot water 60-100° C., this step being necessary for the purpose of removing the adhering polyvinyl alcohol and also for the purpose of shrinking and relaxing the treated polyurethane elastic filaments. By this hot water treatment practically all of the adhering polyvinyl alcohol is removed and a shrinkage of 20-80% is imparted to the woven or knitted product, thus yielding a product abounding in elasticity. One advantage of the method of the present invention is that it is easily attainable to make polyurethane continuous elastic filaments have lower elongation and high Young's modulus by subjecting the filaments to a treatment with an aqueous solution of polyvinyl alcohol whose cost is very cheap. This results in an easy control of polyurethane continuous elastic filaments during the steps of twisting and

the like, while such control is very difficult in the conventional arts.

Another advantage of the method of the present invention is that it is made possible to prepare knitted and woven articles having such a uniform and beautiful appearance as is never seen in the conventional articles by subjecting those articles composed of hard fiber yarns and said polyurethane continuous elastic filaments having a low elongation and being made easily controllable to such a simple step as that of removing polyvinyl alcohol adhered to the articles with hot water.

One skilled in the art can easily attain said advantages and others by following the method of the present invention.

The following non-limitative examples are given for further illustrating the invention.

#### EXAMPLE 1

The three components of polyethylenepropylene adipate having a terminal hydroxyl radical and of a molecular weight of 2000 (ethylene glycol:propylene glycol mole ratio=9:1), diphenylmethane 4,4'-diisocyanate and ethylene glycol were mixed in a molar ratio of 1:5:4, to which was then added 15% by weight of dimethylformamide as solvent to 85% by weight of this mixture. The mixture was reacted for 6 hours at 90° C. and a powdery polyurethane polymer was obtained. This was followed by the incorporation as antioxidants in the so obtained polymer of 1% by weight of 4,4'-butylidenebis(3-methyl-6-tertiarybutyl phenol) and 1.5% by weight of titanium dioxide, based on the polyurethane polymer. This was then dissolved in dimethylformamide to prepare a 28% (wt.) spinning solution.

This spinning solution was extruded from a spinning nozzle having 10 holes, each 0.25 mm. in diameter, into a stream of N<sub>2</sub> gas, following which the freshly spun filaments were dried and then wound up at 350 meters per minute. The so obtained filaments had a denier of 138, a tenacity of 1.08 grams per denier, an elongation of 475% and a Young's modulus (expressed in terms of tenacity at 50% elongation) of 0.08 gram per denier. These elastic filaments were drawn 300% at 140° C. and, while still in their stretched state, were heat treated for 30 seconds in a 15% (wt.) aqueous solution of polyvinyl alcohol having a degree of polymerization of 1000 and a degree of saponification of 88.8%, heated to 95° C., following which the filaments, while still in their stretched state, were dried and thereafter imparted a mechanical shrinkage of 8% to obtain the treated elastic filaments. These treated elastic filaments had a polyvinyl alcohol adhesion of 43% (wt.), a denier of 51, a tenacity of 3.82 grams per denier, an elongation of 64%, and a Young's modulus of 1.87 grams per denier, and they had a high degree of form stability even under free tension.

Next, using the conventional twisting machine, a twisting yarn having a Z twist of 250 turns per meter was obtained from the three yarns of the aforesaid treated elastic yarn 51/1, wooly nylon 70/1 S twist and wooly nylon 70/1 Z twist, without stretching the treated elastic filaments hardly at all. When the so obtained yarn was unreeled from the pirl and allowed to stand under free tension, it showed little, if any, shrinkage and thus had form stability to a high degree.

To so obtained twisting yarn was then used as the warp and a mixed yarn of polyester fiber and rayon [mixture ratio of 50:50 (wt.)] was used as the weft, and a 2/2 twill weave fabric was woven. The width of the resulting fabric was 97 cm. When the polyvinyl alcohol removal and shrinkage treatment of this fabric was carried out for 30 minutes in 90° C. hot water, a 47% shrinkage took place in the longitudinal direction containing the treated elastic yarn. After it was given a finishing treatment, a longitudinally elastic fabric having a fine and uniform surface condition and an extensibility of 42% in the longitudinal direction was obtained.

#### Comparison

5 The treated elastic filaments which were treated exactly as in Example 1 but without the polyvinyl alcohol treatment had a denier of 35, a tenacity of 2.2 grams per denier, an elongation of 190% and a Young's modulus of 0.19 gram per denier. It was thus found that a temporary lowering of the elongation and a temporary raising of the Young's modulus such as intended by the invention were not achieved.

#### EXAMPLE 2

Polyurethane elastic filaments were obtained by dry-spinning, as in Example 1, a polyurethane polymer obtained by mixing polyethylene adipate (molecular weight 1900), diphenylmethane 4,4'-diisocyanate and ethylene glycol in a molar ratio of 1:5:4. The so obtained elastic filaments had a denier of 140, a tenacity of 1.2 grams per denier, an elongation of 530% and a Young's modulus of 0.13 gram per denier.

20 Next, these elastic filaments were drawn 300% in a 23% aqueous solution (18° C.) of polyvinyl alcohol having a degree of polymerization of 1800 and a degree of saponification of 92% followed by allowing to stand 25 therein for 6 seconds. The filaments were then taken out, submitted to a dry heat treatment for 20 seconds at 60° C. in their stretched state and thereafter cooled at room temperature to obtain treated elastic filaments. These filaments had a polyvinyl alcohol adhesion of 70%, a denier of 61, a tenacity of 3.5 grams per denier, an elongation of 80% and Young's modulus of 1.2 grams per denier.

25 Next, a 36s core yarn was made by means of a spinning frame from the foregoing treated elastic filaments and two ends of a slab yarn composed of 65% by weight of polyester staples of 2 denier and 51 mm. fiber length and 35% by weight of rayon staples of 2 denier and 51 mm. fiber length. The core yarn was spun under the conditions of a spindle speed of 3000 r.p.m., 720 twists per meter, a twist multiplier of 3.0, a front roller diameter of 28.5 mm. and a front roller speed of 47.3 r.p.m. The cone-wound treated elastic filaments were unwound from the cone longitudinally thereof and were positioned in the middle of the slab yarns in a practically unstretched state, and the core yarn was made without application of 30 a draft. The so obtained core yarn demonstrated little, if any, extensibility. These conditions which were employed in this example for spinning the core yarn are those which are usually used when making a core yarn from hard fiber yarns.

35 Next, a fabric was woven using a mixed yarn of polyester and rayon fibers as the warp and in alternation the core yarn and a mixed yarn of polyester and rayon fibers as the weft. In this case, the core yarn was maintained in a practically unstretched state during the weaving process. The resulting fabric demonstrated practically no extensibility, and when the 200-cm. wide fabric was treated 40 in 85° C. hot water for 30 minutes, it shrunk to a width of 140 cm. After drying, the fabric had a uniform surface condition, and it was a laterally elastic fabric demonstrating an extensibility of 25% in the lateral direction.

#### EXAMPLE 3

An isocyanate-terminated polyester was obtained by 45 reacting one mol of polyethylene adipate (molecular weight 2410) with 2 moles of 2,4-tolylene diisocyanate, following which the resulting polyester was dissolved in dimethylacetamide. This was followed by reacting the isocyanate-terminated polyester in dimethylacetamide with 50 an equivalent of ethylene diamine to obtain a polyurethane polymer. This polymer was dissolved in dimethylacetamide to prepare a 20% solution of the polymer, which was then wet-spun into a 70° C. water bath to obtain 55 a polyurethane elastic filaments having a denier of

155, a tenacity of 1.02 grams per denier, an elongation of 638% and a Young's modulus of 0.09 gram per denier.

Next, these elastic filaments were drawn 850% while spraying it with a 26% aqueous solution (23° C.) of polyvinyl alcohol having a degree of polymerization of 1750 and a degree of saponification of 98%, following which the filaments were submitted to a dry heat treatment for 23 seconds at 72° C. in their stretched state and thereafter air dried to obtain treated elastic filaments. These filaments whose polyvinyl alcohol adhesion was 125% had a denier of 47, a tenacity of 2.2 grams per denier, and elongation of 95% and a Young's modulus of 0.42 gram per denier.

Next, employing the spinning frame used in Example 2 and with the spinning conditions used therein, a 42s core yarn was made from the foregoing treated elastic filaments and 3 ends of slub yarns composed of 60% by weight of polyacrylonitrile staples of 4 denier and 30 mm. fiber length and 40% by weight of rayon staples of 4 denier and 30 mm. fiber length.

A fabric was then woven using as the warp a mixed yarn of polyacrylonitrile fiber and rayon (mixture ratio = 50:50) and as the weft the aforesaid core yarn and the mixed yarn of polyacrylonitrile fiber and rayon in alternation. The fabric obtained demonstrated practically no extensibility. When this fabric whose width was 175 cm. was treated for 22 minutes in 90° C. hot water, it shrank to 125 cm. After drying, the fabric became a laterally elastic fabric having an extensibility of 27% in the lateral direction.

#### EXAMPLE 4

One mole of a polyetherester glycol of a molecular weight of 2600 obtained from sebacic acid and diethylene glycol and 2.1 moles diphenylmethane 4,4'-diisocyanate were heated for one hour at 93° C., then dissolved in dimethylacetamide, after which an equimolar amount of water was added and the mixture was reacted for 5 hours at 93° C. A 20% dimethylacetamide solution of the so obtained polyurethane elastomer was prepared and dry-spun as in Example 1. The resulting filaments had a denier of 130, a tenacity of 1.02 grams per denier, an elongation of 510% and a Young's modulus of 0.1 gram per denier. These elastic filaments were treated in a 13% aqueous solution (15° C.) of polyvinyl alcohol having a degree of polymerization of 1300 and a degree of saponification of 87%, after which the filaments were removed from the foregoing aqueous solution and drawn 300% in customary manner, dried for 25 seconds at 75° C. in their stretched state, and thereafter cooled at room temperature to obtain treated elastic filaments, which had a polyvinyl alcohol adhesion of 77%, a denier of 41, a tenacity of 2.9 grams per denier, an elongation of 93% and a Young's modulus of 0.95 gram per denier.

These filaments were submitted to a doubling and twisting operation as in Example 1 to obtain a 210 twists per meter Z twist twisting yarn. A 2/2 twill weave fabric was woven using this yarn as the warp and a mixed yarn of polyester fiber and rayon as the weft. The width of the resulting fabric was 150 cm. When this fabric was heat treated for 20 minutes in hot water (91° C.), the polyvinyl alcohol was removed and at the same time a shrinkage of 31% took place in the warp direction. The resulting fabric had an extensibility of 21% in the longitudinal direction.

#### EXAMPLE 5

The undrawn, still unheat-treated elastic filaments obtained in Example 1, having a denier of 138, a tenacity of 1.08 grams per denier, an elongation of 475% and a Young's modulus of 0.08 gram per denier were drawn 350% in a 12% aqueous solution (90° C.) of polyvinyl alcohol having a degree of polymerization of 2500 and a degree of saponification of 95% followed by heat treating for 15 seconds to obtain treated elastic filaments. The

so obtained treated elastic filaments had a polyvinyl alcohol adhesion of 18%, a denier of 46, a tenacity of 18 grams per denier, an elongation of 66% and a Young's modulus of 1.48 grams per denier. They possessed a high degree of form stability even under free tension and demonstrated practically no extensibility. These treated elastic filaments and a 50 denier yarn of polyamide fiber (nylon) were warped by means of a tricot warper with the treated elastic filaments in a practically unstretched state and then wound up on two sets of beams. Guides were provided in two places during the warping step but practically no tension irregularities ascribable to the guides appeared in the treated elastic filaments. Next, a tricot knitting machine was used and a half tricot having a machine width of 280 cm. was made, the design being such that the nylon would be in the front while the treated elastic filaments would be in the back. It was possible to carry out this knitting operation quite smoothly. The so obtained half tricot was treated for 30 minutes in a 70° C. water bath containing "Scourol" (a nonionic surfactant of polyethylene glycol ether, a product of Kao Soap Company, Japan) as the scouring agent, then treated for 15 minutes in 100° C. boiling water containing "Scourol," followed by washing in 60° C. hot water, drying for one minute at 100° C. at a constant length and thereafter setting for one minute at 170° C. at a constant length to obtain a 165-cm.-wide product. As compared with the product in which only nylon was used, this product had a soft feel and fine appearance as well as an extensibility of 59%. No irregularities ascribable to the tension irregularity of the elastic filaments could be observed in this product.

I claim:

1. A method of producing an elastic fabric which consists essentially of applying to the surface of polyurethane continuous elastic filaments an aqueous temporary setting solution of polyvinyl alcohol having a degree of saponification of 50-100% and subjecting the filaments to drying under a stretched state ranging from at least 150 percent of the original length of said filaments to below the breaking elongation thereof to thereby obtain polyurethane continuous elastic filaments of low elongation coated with said polyvinyl alcohol whose elongation is not greater than 100% and whose Young's modulus as expressed in terms of tenacity in grams per denier at 50% elongation is at least 0.4 gram per denier, and thereafter making a fabric using the thus obtained filaments with hard fiber yarns, followed by treating the resulting fabric in hot water of 60-100° C. to remove the polyvinyl alcohol setting solution from the surface of said polyurethane filaments thus yielding an elastic fabric.
2. The method according to claim 1 wherein said aqueous solution of polyvinyl alcohol is a concentration of 1-30 percent by weight and the amount applied of said polyvinyl alcohol is 5-200 percent by weight based on the filaments.
3. The method according to claim 1 wherein the polyvinyl alcohol is adhered to the surface of said polyurethane continuous elastic filaments by dipping said filaments in said polyvinyl alcohol aqueous solution.
4. The method according to claim 1 wherein the temperature of said polyvinyl alcohol aqueous solution to be applied is 100° C.
5. The method according to claim 1 wherein the polyurethane continuous elastic filaments are concurrently subjected to drying and heat treatment by using a drying temperature of 60-100° C.
6. The method according to claim 1 which comprises exposing said polyurethane continuous elastic filaments in their stretched state to a temperature ranging from 60° C. to a temperature just below the decomposition temperature of said filaments during a period before the completion of the drying of the polyvinyl alcohol applied to said polyurethane continuous elastic filaments.

7. The method according to claim 1 wherein said hard fiber yarns are yarns which have been subjected to a bulking treatment.

3,093,504 6/1963 Bode ----- 28—75  
3,227,192 4/1966 Griffiths ----- 28—75 X

## FOREIGN PATENTS

## References Cited

## UNITED STATES PATENTS

2,157,463 5/1939 Shepherd.  
2,427,334 9/1947 Alderfer.  
2,852,834 9/1958 Engelhard.

5 710,507 6/1965 Canada.  
552,190 3/1943 Great Britain.  
LOUIS K. RIMRODT, Primary Examiner  
U.S. Cl. X.R.  
10 28—76